

# United States Patent Office

3,038,820

Patented June 12, 1962

1

3.038.820

5,938,620

# PROCESS FOR IMPARTING A SOFT FEEL TO TEXTILE FIBERS

Otto Albrecht, Munchenstein, Switzerland, assignor to  
Ciba Limited, Basel, Switzerland  
No Drawing. Filed Mar. 23, 1959, Ser. No. 800,968  
Claims priority, application Switzerland July 15, 1955  
9 Claims. (Cl. 117—139.5)

The present application is a continuation-in-part of my application Serial No. 666,782, filed June 19, 1957, which is a division of my copending application Serial No. 596,444, filed July 9, 1956 (both of which applications are now abandoned).

This invention provides a new process for imparting a soft feel to organic textile fibers which comprises applying to said fibers in an aqueous bath a polyglycol ether derivative, in which each carbon atom bound to an oxygen atom is bound to a single oxygen atom, and which contains the radical of an amine of the formula



in which  $m$  represents a small whole number, and in which there are bound to nitrogen atoms of the amine radical at least two acyl radicals together containing at least 20 carbon atoms and derived from fatty acid.

The aforesaid polyglycolether derivative can be made by introducing a polyglycol ether chain, advantageously with the aid of ethylene oxide, into an acyl-compound which is derived from an amine of the Formula 1 and contains at least two acyl radicals which are derived from fatty acids and together contain at least 20 carbon atoms, and in which acyl compound each carbon atom bound to an oxygen atom is bound to a single oxygen atom.

Particularly, this invention provides a process for imparting a soft feel to organic textile fibers which comprises treating said fibers with an aqueous bath which contains a compound which in its free base state is a reaction product of 8-30 mols of ethylene oxide and 1 mol of an N-acylated alkylene polyamine which contains 2 to 4 nitrogen atoms separated from each other by alkylene groups containing 2 to 3 carbon atoms, in which N-acylated alkylene polyamine at least 2 nitrogen atoms are acylated by a saturated aliphatic monocarboxylic acid containing 12 to 18 carbon atoms, and drying the fibers.

As starting materials for making the ethylene oxide reaction products there may be used, for example, amines of the kind defined above which are diacylated with fatty acids, advantageously acylamino-compounds of the formula



in which the radicals  $R_1$  are saturated aliphatic hydrocarbon radicals containing 1-17 carbon atoms,  $n$  represents an integer from 1 to 2,  $m$  represents an integer from 1 to 3,  $p$  is an integer from 2 to 4 and is greater than  $m$  by at most 1, and the radicals  $-\text{CO}-R_1$  together contain at least 20 carbon atoms.

More particularly, there may be used N-acylamino compounds corresponding to the general formula

2

wherein  $n$ ,  $p$ ,  $q$ ,  $k$  and  $m$  each represent an integer from 1 to 2,  $R_1$ ,  $R_2$ ,  $R_3$  and  $R_4$  each represent a saturated aliphatic hydrocarbon radical containing 1 to 7 carbon atoms, at least two of the acyl radicals containing 12 to 18 carbon atoms each.

The acyl-compounds are derived from aliphatic alkylene polyamines which contain 2 to 4 nitrogen atoms separated from each other by at least one divalent alkylene group containing 2 to 3 carbon atoms, preferably by at least one ethylene group, for example, from ethylene diamine, propylene diamine, diethylene triamine or triethylene tetramine. Especially advantageous are the acyl compounds of diethylene triamine. The acyl compounds derived from diethylene triamine correspond to the formula



in which  $R_1$  represents a saturated aliphatic hydrocarbon radical containing 1 to 17, preferably 11-17, carbon atoms,  $p$  represents an integer from 2 to 3, and the acyl radicals  $-\text{OC}-R_1$  together contain at least 20 carbon atoms, at least 2 acyl radicals each containing at least 8 carbon atoms.

25 Still more particularly the acyl compounds derived from diethylene triamine correspond to the formula



wherein  $p$  represents an integer from 1 to 2,  $R_1$ ,  $R_2$  and  $R_3$  each represent a saturated aliphatic hydrocarbon radical containing 1 to 17 carbon atoms, at least two of the acyl radicals containing 12 to 18 carbon atoms each.

The acyl compounds used as starting materials for making the polyglycol ether derivatives therefore contain at least two N-acyl radicals, the acyl radicals must together contain at least 20 carbon atoms, and it is generally advantageous that there should be present in the molecule at least two acyl radicals each containing at least 8 carbon atoms. Preferably there are used compounds containing the same number of acyl radicals as there are amino groups. These products are present when, for example, *p* in the Formula 4 is 3 and when *p* in the Formula 5 is 1.

The acyl radicals of the compounds of the Formulae 2, 3, 4 and 5 contain from 1 to 22, preferably from 12 to 18, carbon atoms. Accordingly, the acyl radicals are derived, for example, from advantageously unbranched saturated fatty acids of high molecular weight, such as lauric acid (for example, in the form of coconut oil fatty acid), myristic acid, palmitic acid, arachic acid or behenic acid. Especially advantageous are, for example, acyl compounds derived from stearic acid, and especially those of which the acyl radicals are those of so-called commercial stearic acid consisting for the greater part of stearic acid. If the acyl radicals are derived from fatty acids of low molecular weight they consist, for example, of an acetyl, propionyl or butyryl radical.

The acyl-compounds used as starting materials for mak-



ing the polyglycol ether derivatives can be prepared in known manner from the appropriate polyamines and carboxylic acids, or, if desired, functional derivatives of these acids, such as their acid halides, especially their acid chlorides, or acid anhydrides. When acyl radicals of low molecular weight are introduced in addition to acyl radicals of high molecular weight, it is of advantage to introduce the former acyl radicals last.

The acylamino-compounds are reacted with ethylene oxide advantageously at a raised temperature with the exclusion of atmospheric oxygen and preferably in the presence of a suitable catalyst, for example, a small quantity of an alkali metal or alkali metal hydroxide, carbonate or acetate.

The amount of additively combined ethylene oxide is critical. Useful softening agents are obtained when 1 mol of the acylamino-compound is reacted with about 8-30, advantageously about 15-20 mols of ethylene oxide. In general these products possess good resistance to heat and have little or no yellowing affinity on the textile fibers treated therewith. When applied to dyed material, the fastness to light of the dyeing is usually not impaired at all or only to an inconsiderable extent. The polyglycol ether compounds are very suitable for incorporation in anti-creasing treatment baths, so as to impart to the treated material an anti-crease resistant dressing and also a soft feel.

From the foregoing description it will be apparent that especially valuable softening agents are the products of the formula



in which the radicals  $R_1$  are saturated aliphatic hydrocarbon radicals containing 1-17, preferably 11-17 carbon atoms and the radicals —A corresponds to the formula



(in which  $k$  is a whole number),  $p$  is an integer from 2 to 3, and the radicals  $-\text{OC}-\text{R}_1$  together contain at least 20 carbon atoms at least two of these radicals each containing at least 8 carbon atoms, and the molecule of the product contains about 8-30  $-\text{CH}_2-\text{CH}_2-\text{O}-$  groups.

Still more particularly the invention provides a process for imparting a soft feel to organic textile fibers which comprises treating said fibers with an aqueous solution of a compound which in its free base state corresponds to the general formula



wherein  $p$  represents an integer from 1 to 2,  $k$ ,  $r$  and  $s$  each represents an integer from 1 to 29, the sum of  $k+r+s$  being at least 8 and at the most 30, and  $R_1$ ,  $R_2$  and  $R_3$  each represent a saturated aliphatic hydrocarbon radical containing 1 to 17 carbon atoms, at least two of these acyl radicals containing 12 to 18 carbon atoms each, the treated fibers containing said compound in an amount of 0.08-1.2, preferably of 0.1-1 percent, calculated on the weight of the fibers, and drying the fibers at elevated temperatures.

Those polyglycol ether derivatives which contain at least one basic nitrogen atom can be converted in known manner into salts, for example, acetates, or, if desired, into quaternary ammonium salts, and used in this form. In the process of the invention there are treated synthetically produced or chemically modified cellulosic fibers or regenerated cellulosic fibers the manufacturing process of which has been completed. Synthetically

produced fibers to be subjected to the process of this invention are those of polyacrylonitrile, polyesters, polyamides or polyurethanes; chemically modified cellulosic fibers are those of cellulose acetate or cellulose ether; and regenerated cellulosic fibers are those of rayon. Besides these synthetically produced or semi-synthetically produced fibers there come into consideration animal fibers, such as wool or silk and natural cellulosic fibers, such as cotton or linen. Especially good softening effects are obtained by treating fibers from polyacrylonitrile, polyamides, rayon and cellulose triacetate.

The aqueous treating bath contains the described softening agents in such an amount that the treated fibers may contain 0.08 to 1.2, preferably 0.1 to 1 or 0.15 to 0.8 percent of the softening agent. The fibers may be treated with the bath in the usual exhaust process or by the padding process.

When, in the exhaust process, polyacrylonitrile, polyester, polyamide, or cellulose acetate fibers are to be treated, the bath contains 0.1–0.2 percent of the softening agent; in the case of cotton it contains about 0.2–0.4; and in the case of wool fibers about 0.8–1.2 percent, calculated on the weight of the fibers.

The temperature of the treating bath may vary within wide limits, for example, between 20° C. and 100° C. As a rule, the fibers are treated at temperatures between 20 and 40° C. After the treating with the bath the fibers are dried, usually without previous rinsing, at temperatures ranging from 20 to 160° C., preferably at elevated temperatures i.e. at a temperature between 60 and 120° C.

The following examples illustrate the invention, the parts and percentages being by weight:

### *Example 1*

35 Defatted yarn of viscose artificial silk is worked at a liquor ratio of 1:30 for  $\frac{1}{2}$  hour at  $20^{\circ}\text{ C}$ . in a solution, prepared with water of  $20^{\circ}$  German hardness and containing 0.1 percent of the condensation product (a), (b) or (c) described below, calculated on the weight of the 40 yarn. After separating the excess of liquor and drying the material, the yarn so treated has a soft slippery feel.

(a) 103 parts (1 mol) of diethylene triamine are heated in a current of nitrogen to 140° C. under a descending condenser, and 540 parts (2 mols) of commercial stearic acid are added in the course of 4 hours. The mixture is stirred for a further 4 hours in a current of nitrogen at 160–165° C. One molecular proportion of the condensation product so obtained is then reacted with 25 molecular proportions of ethylene oxide at 110–130°

C. in the presence of about 1 percent of sodium calculated on the acylation product. The polyglycol ether derivative is a soft mass which is easily soluble in water.

(b) 92.7 parts (1 molecular proportion) of diethylene triamine and 729 parts (3 molecular proportions) of commercial stearic acid are heated in a current of nitrogen at 140° C., and then the mixture is first heated for 3 hours at 140–145° C. and thereafter for a further 4½ hours at 160–165° C. Nitrogen is continuously passed through the apparatus. There are obtained 776 parts of a pale wax-like condensation product.

60 parts (1 molecular proportion) of the reaction product so obtained are melted in a current of nitrogen, then 0.15 part of sodium is added, and ethylene oxide is introduced as a finely distributed gas stream at 150–160° C. until 92 parts (30 molecular proportions) of ethylene oxide have been taken up. The hydroxyethylation product so obtained is a light colored solid mass, which yields

(c) 92.7 parts (1 molecular proportion) of diethylene triamine and 729 parts (3 molecular proportions) of commercial stearic acid are heated in a current of nitrogen to 140° C., and then the mixture is first heated for 3 hours at 140–145° C. and then for a further 4½ hours at 160–165° C. Nitrogen is continuously passed through the apparatus. There are obtained 776 parts of a pale wax-like condensation product.

60 parts (1 molecular proportion) of the reaction product so obtained are melted in a current of nitrogen, and then 0.15 part of sodium is added and ethylene oxide is introduced as a finely distributed gas stream at 150–160° C. until 46 parts (15 molecular proportions) of ethylene oxide have been taken up. In this manner the hydroxyethylation product is obtained in the form of a light colored solid mass which when taken up in warm water yields an opalescent solution.

*Example 2*

100 parts of defatted yarn of viscose artificial silk are treated for  $\frac{1}{2}$  hour at  $20^\circ$  C. in a solution containing 0.3 part of the acetate (*d*) (50 percent amine content) described below in 3000 parts of distilled water. This treatment imparts a soft feel to the yarn.

A similar result is obtained by treating the yarn on a foulard with a solution containing 2.5 grams of the aforesaid acetate in one liter of water.

(d) The acetate of the condensation product (a) described above in Example 1 can be prepared by mixing 15 parts of the condensation product with 4.4 parts of acetic acid of 20 percent strength and 10.6 parts of water. In this manner there is obtained a paste having a calculated content of 50 percent of amine.

### Example 3

100 parts of fibers of polyacrylonitrile are treated for 20-30 minutes at 20° C. in a solution containing 0.15 part of the softening agents (e), (f), (g) or (h) described below in 3000 parts of water. The fibers are dried, without rinsing, at temperatures between 60-80° C. This treatment imparts a soft feel to the yarn.

(e) 103 parts (1 mol) of diethylene triamine are heated to 140° C. in a current of nitrogen, and 540 parts (2 mols) of commercial stearic acid are added in small portions in the course of 4 hours. The whole is then stirred for a further 4 hours at 160–165° C. Throughout the reaction nitrogen is passed through the apparatus continuously in order to prevent discoloration as far as possible.

121.4 parts (1 molecular proportion) of the condensation product so obtained are melted in a boiling water bath and 22.4 parts (1 molecular proportion) of acetic anhydride are run in the course of one hour. The whole is then stirred for 2 hours in a boiling water bath. The reaction product is then treated with a dilute solution of sodium carbonate, taken up in an organic solvent, and then freed from solvent.

20 parts (1 molecular proportion) of the acylation product so obtained are melted in a current of nitrogen, 0.2 part of metallic sodium is added, and ethylene oxide is introduced in a finely distributed gas stream at 160-170° C. until 13.5 parts (10 molecular proportions) of ethylene oxide have been absorbed. In another sample, 20 parts of the acylation product are reacted with 10.8 parts (8 molecular proportions) of ethylene oxide. The

ethoxylation products are solid masses, which are almost clearly soluble in warm water.

(f) Diethylene triamine is diacylated in commercial stearic acid as described in the first paragraph of Example 1. 80 parts (1 molecular proportion) of the resulting distearyl diethylene triamine (from commercial stearic acid) are melted in a current of nitrogen, and then 0.8 part of sodium is added and ethylene oxide is introduced as a finely distributed gas stream until 180 parts (18 molecular proportions) thereof have been taken up. The condensation product, which is a rather soft mass, is soluble in water.

(g) 243 parts (3 molecular proportions) of commercial stearic acid are heated in a current of nitrogen until they melt, and 43.8 parts (1 molecular proportion) of triethylene tetramine are added to the melt having a temperature of about  $110^{\circ}\text{ C}$ . The reaction mass is then heated at  $140$ – $145^{\circ}\text{ C}$ . for 3 hours, and then at  $160$ – $165^{\circ}\text{ C}$ .

heated at 140–145°C. for 3 hours, and then at 160–165°C. for 4½ hours with stirring. During this time nitrogen is passed through the apparatus.

100 parts (1 molecular proportion) of the condensation product so obtained are heated to 150° C. in a current of nitrogen, whereupon ethylene oxide is introduced as a finely distributed gas stream until 109.4 parts (22 molecular proportions) are taken up. The resulting polyglycol ether derivative is a wax-like mass which is soluble in water.

(h) 74 parts of propylene diamine (1 mol) and 540 parts (2 mol) of commercial stearic acid are heated to 140° C. in a current of nitrogen, whereupon the reaction mass is heated first at 140–145° C. for 3 hours and then at 160–165° C. for 4 hours. During this time, nitrogen is passed through the apparatus. 60 parts (1 molecular proportion) of the reaction product so obtained are melted in a current of nitrogen, and 0.15 part of sodium added, and at 150–160° C. ethylene oxide is introduced as a finely distributed gas stream until 70 parts (15 molecular proportions) are taken up.

*Example 4*

40 Fibers mentioned in the table below are worked at a  
 liquor ratio of 1:30 for 10-30 minutes at a temperature  
 between 30-55° C. in a solution containing the indicated  
 percentage of condensation product (c) of Example 1,  
 45 calculated on the weight of the fibers. The textile fibers  
 are dried, without rinsing, at temperatures from 60-80° C.

| Fiber:                | Percent softening agent |
|-----------------------|-------------------------|
| Polyacrylonitrile     | 0.15                    |
| 50 Polyester          | 0.15                    |
| Polyamide             | 0.15                    |
| Cellulose-2½-acetate  | 0.15                    |
| Cellulose-tri-acetate | 0.15                    |
| Rayon                 | 0.08                    |
| 55 Cotton             | 0.3                     |
| Wool                  | 1.2                     |

Especially good softening results are obtained with fibers of cellulose-tri-acetate and also with fibers of poly-acrylonitrile, polyamides and rayon.

60 What is claimed is:

1. A process for imparting a soft feel to organic textile fibers which comprises treating said fibers with an aqueous solution of a compound which in its free base state is a reaction product of 10-25 mols of ethylene oxide and 1-65 mol of an N-acylated alkylene polyamine which corresponds to the formula



wherein  $n$ ,  $p$ ,  $q$ ,  $k$  and  $m$  each represent an integer from 1 to 2,  $R_1$ ,  $R_2$ ,  $R_3$  and  $R_4$  each represent a saturated aliphatic hydrocarbon radical containing 1 to 17 carbon atoms, at least two of the acyl radicals containing 12 to 18 carbon atoms each, the treated fibers containing said reaction product in an amount of 0.08-1.2 percent, calculated on the weight of the fibers, and drying the fibers at elevated temperatures.

2. A process for imparting a soft feel to organic textile fibers which comprises treating said fibers with an aqueous solution of a compound which in its free base state is a reaction product of 10-25 mols of ethylene oxide and 1 mol of an N-acylated alkylene polyamine which corresponds to the general formula



wherein  $n$ ,  $p$  and  $k$  each represent an integer from 1 to 2,  $R_1$ ,  $R_2$  and  $R_3$  each represent a saturated aliphatic hydrocarbon radical containing 1 to 17 carbon atoms and, at least two of the acyl radicals containing 12 to 18 carbon atoms, the treated fibers containing said reaction product in an amount of 0.08-1.2 percent, calculated on the weight of the fibers, and drying the fibers at elevated temperatures.

3. A process for imparting a soft feel to organic textile fibers which comprises treating said fibers with an aqueous solution of a compound which in its free base state is a reaction product of 10-25 mols of ethylene oxide and 1 mol of an N-acylated alkylene polyamine which corresponds to the general formula



wherein  $p$  represents an integer from 1 to 2,  $R_1$ ,  $R_2$  and  $R_3$  each represent a saturated aliphatic hydrocarbon radical containing 1 to 17 carbon atoms each, at least two of the acyl radicals containing 12 to 18 carbon atoms, the treated fibers containing said reaction product in an amount of 0.08-1.2 percent, calculated on the weight of the fibers, and drying the fibers at elevated temperatures.

4. A process for imparting a soft feel to organic textile fibers selected from the group consisting of animal fibers, cellulosic fibers and synthetic fibers which comprises treating said fibers with an aqueous solution of a compound which in its free base state is a reaction product of 10-25 mols of ethylene oxide and 1 mol of an N-acylated alkylene polyamine which corresponds to the general formula



wherein  $R_1$  and  $R_2$  each represent a saturated aliphatic hydrocarbon radical containing 11-17 carbon atoms, the treated fibers containing said reaction product in an amount of 0.08-1.2 percent, calculated on the weight of the fibers, and drying the fibers at elevated temperatures.

5. A process for imparting a soft feel to organic textile fibers selected from the group consisting of animal fibers, cellulosic fibers and synthetic fibers which comprises treating said fibers with an aqueous solution of a compound which in its free base state is a reaction product of 10-25 mols of ethylene oxide and 1 mol of an N-acylated alkylene polyamine which corresponds to the general formula



wherein  $R_1$ ,  $R_2$  and  $R_3$  each represent a saturated aliphatic hydrocarbon radical containing 11-17 carbon atoms, the treated fibers containing said reaction product in an amount of 0.08-1.2 percent, calculated on the weight of the fibers, and drying the fibers at elevated temperatures.

6. A process for imparting a soft feel to organic textile fibers selected from the group consisting of animal fibers, cellulosic fibers and synthetic fibers which comprises treating said fibers with an aqueous solution of a compound which in its free base state is a reaction product of 10-25 mols of ethylene oxide and 1 mol of an N-acylated alkylene polyamine which corresponds to the formula



the treated fibers containing said reaction product in an amount of 0.1-1 percent, calculated on the weight of the fibers, and drying the fibers at elevated temperatures.

7. A process for imparting a soft feel to organic textile fibers selected from the group consisting of animal fibers, cellulosic fibers and synthetic fibers which comprises treating said fibers with an aqueous solution of a compound which in its free base state is a reaction product of 10-25 mols of ethylene oxide and 1 mol of an N-acylated alkylene polyamine which corresponds to the formula



the treated fibers containing said reaction product in an amount of 0.1-1 percent, calculated on the weight of the fibers, and drying the fibers at elevated temperatures.

8. A process for imparting a soft feel to cellulose triacetate fibers which comprises treating said fibers with an aqueous solution of a compound which in its free base state is a reaction product of 15 mols of ethylene oxide and 1 mol of an N-acylated alkylene polyamine which corresponds to the formula



the treated fibers containing said reaction product in an amount of 0.1-1 percent, calculated on the weight of the fibers and drying the fibers at elevated temperatures.

9. A process for imparting a soft feel to cellulose triacetate fibers which comprises treating said fibers with an aqueous solution of a compound which in its free base state is a reaction product of 15 mols of ethylene oxide and 1 mol of an N-acylated alkylene polyamine which corresponds to the formula



the treated fibers containing said reaction product in an amount of 0.1-1 percent, calculated on the weight of the fibers and drying the fibers at elevated temperatures.

#### References Cited in the file of this patent

#### UNITED STATES PATENTS

|           |                        |               |
|-----------|------------------------|---------------|
| 1,924,698 | Neelmeier et al. ----- | Aug. 29, 1933 |
| 2,085,706 | Schoeller et al. ----- | June 29, 1937 |
| 2,103,872 | Schoeller et al. ----- | Dec. 28, 1937 |
| 2,201,041 | Katz -----             | May 14, 1940  |
| 2,340,881 | Kelly et al. -----     | Feb. 8, 1944  |
| 2,596,985 | Cook et al. -----      | May 20, 1952  |
| 2,681,354 | Kelly et al. -----     | June 15, 1954 |
| 2,901,430 | Chiddix et al. -----   | Aug. 25, 1959 |